

April 6, 1965

E. BÖCKLY ET AL

3,177,078

FILTER AND ABSORBING DYES FOR PHOTOGRAPHIC EMULSIONS

Filed Jan. 21, 1963

FIG.1



FIG.2

INVENTORS:

ERICH BÖCKLY, KARL LÖFFLER, REINHARD MÜLLER.

BY Connolly and Aus  
then ATTORNEYS

1

3,177,078  
FILTER AND ABSORBING DYES FOR PHOTOGRAPHIC EMULSIONS

Erich Böckly, Cologne-Stammheim, Germany, Karl Löffler, deceased, late of Leverkusen, Germany, by Beate Löffler, legal representative, Leverkusen, Germany, and Reinhard Müller, Leverkusen, Germany, assignors to Agfa Aktiengesellschaft, Leverkusen, Germany, a corporation of Germany

Filed Jan. 21, 1963, Ser. No. 253,003

Claims priority, application Germany, Feb. 3, 1962,  
A 39,366  
6 Claims. (Cl. 96—74)

This invention relates to photographic silver halide emulsions containing light-absorbing additives and photographic elements comprising layers of such emulsions.

The sharpness and resolution of photographic images produced with photosensitive layers of silver halide emulsions are impaired by the light scattering caused by the silver halide grains. This effect can be reduced by colouring the photosensitive layers with dyestuffs which absorb light in the spectral range to which the emulsion is sensitive, which dyestuffs may then be removed after exposure. The harmful effect of the scattered light is attenuated owing to the longer path which the light has to traverse than the light which falls directly on the silver halide granules to produce the image.

The increased sharpness of definition that can be obtained with these absorbing dyestuffs is inevitably associated with a reduction in the photographic sensitivity.

Dyestuffs which still further reduce the sensitivity of the emulsion layers by virtue of their desensitising properties are of course unsuitable.

Dyestuffs, particularly when used for colour photography, must be practically completely decolorised or removed subsequently because even a faint stain of residual dyestuff can considerably impair the quality of a colour image. Many dyestuffs which are decolorised by the agents used in the processing baths, e.g., by sodium sulphite or potassium ferricyanide are useless because mostly the decolorisation is incomplete. It is therefore advantageous to use dyestuffs which can be washed out of gelatine layers.

Dyestuffs which are suitable for absorbing the scattered light particularly in the red sensitive layer of multiple layer photographic materials without having a desensitising action and which may be removed quantitatively from gelatine layers by washing with water are by far rarer than absorbing dyestuffs for the layers which are sensitive to green or blue.

In French patent specification 1,163,100, dyestuffs are proposed as additives which are prepared by sulphonation of aminoanthraquinone derivatives. The dyestuffs can be washed out of photographic gelatine layers. However, these protective dyestuffs do not adequately absorb in the 680 to 710 m $\mu$  region which is particularly important in multi-layer colour copying materials because the red sensitive layers have the highest sensitivity in this region.

It is among the objects of the present invention to provide for the red sensitive layer dyestuffs which are easily soluble in water, particularly for colour photographic multi-layer copying materials which have a strong absorptive action in the whole red region of the spectrum, especially in the region of maximum red sensitivity, which have practically no desensitising effect on the silver halide emulsion and which can readily be washed out with water in the usual course of processing without requiring any additional baths and without leaving any residual stain.

We have now found that a particular group of dyestuffs can advantageously be employed in red sensitive

2

silver halide emulsions. These blue-green dyestuffs are produced by the action of ferric chloride on sulphonated acids of 1,2-naphthylene diamine. The resulting iron complex dyestuffs, the chemical constitution of which is not completely known in every case, are readily water-soluble and compatible with gelatine-silver halide emulsions and are distinguished by a very wide absorption range which includes the entire red spectrum.

In the region of 620 to 750 m $\mu$  the absorption of these dyestuffs does not fall below 85% of the maximum absorption of about 710 m $\mu$ . The dyestuffs are stable even at very acid or alkaline pH values. Strong reducing agents destroy the iron complexes and causes decolorisation.

The absorbing dyestuffs according to the invention are added in aqueous solution, preferably in quantities of 0.5 to 5 grams per gram atom of silver in the form of silver halide to the gelatine-silver halide emulsions before casting. Based on the quantity of silver halide in the emulsion, we have found that for about 0.5 to about 10 g. of dye per gram mole of silver can be employed, although higher or smaller amounts of dye can be used depending upon particular conditions. Owing to the high water-solubility of the dyestuffs and their low affinity to gelatines they become distributed over adjacent layers so that it may be advantageous to colour not only the red sensitive emulsion layer but also the other emulsion layers before casting. The dyestuffs, which are uniformly distributed in all the layers, in addition reduce the intensity of reflected light.

The preparation and application of the dyestuffs (A, B, C) according to the invention is described in the following examples and the absorption curves of the dyestuffs are shown in FIGURE 1. For comparison, FIGURE 2 shows the spectral distribution of red-sensitivity of the photographic layer sensitised with dyestuff Rr 1953 (Fiat Final Report No. 943), with the main maximum of red sensitisation in the region between 680 and 710 m $\mu$ , which is characteristic for multi-layer copying materials for colour photography.

Rr 1953 conforms to the following formula:



The 1:2-diaminonaphthalene disulphonic acids required in the preparation of the absorbing dyestuffs may be obtained in known manner by coupling diazotised aromatic amino compounds with 2-naphthylamine disulphonic acids in a slightly acidic solution and reductive splitting of the resulting o-aminoazo dyestuffs into 1,2-diamino compounds, e.g., 1:2-diaminonaphthalene-3,6-disulphonic acid from 2-aminonaphthalene-3,6-disulphonic acid (see Beilstein, volume 14, page 793).

60 Example 1

31.8 g. of 1,2-diaminonaphthalene-3,7-disulphonic acid was dissolved by gently heating it in 100 ml. of water and adding 80 ml. saturated sodium acetate solution. 65 32.4 g. of ferric chloride dissolved in 100 ml. of water were then gradually added with stirring at 30° C. to the yellow solution. After allowing the mixture to stand at room temperature for one hour, the precipitated dyestuff (A) was isolated by suction filtering and digested twice with a small quantity of 15% hydrochloric acid and then filtered by suction until dry in air and subsequently completely dried at 70°. 12 g. of dark green

powder readily soluble in water to give a clear solution with a brilliant blue-green colour were obtained.

A solution of 0.6 g. of this dyestuff in 30 ml. water was added to 1 kg. of a gelatine-silver chlorobromide emulsion which had been sensitised to red with dyestuff Rr 1953 (Fiat Final Report No. 943) and which also contained 15 g. of the blue green coupling agent 1-oxy-2-naphthoyl-4-sulpho-octadecylamide, the solution of the dyestuff being added in the proportion 3.7 g. dyestuff per gram atom silver.

This emulsion was used for the middle layer of a three layer positive colour film. The lowest layer applied on a cellulose triacetate foil consisted of a blue sensitive gelatine-silver bromide emulsion with yellow colour coupler, and the uppermost layer was a green sensitive gelatine-silver chlorobromide emulsion with magenta colour coupler. The layers contained about 42 mg. of dyestuff (A) per m.<sup>2</sup>. For comparison, the same three layer film was composed without the addition of absorbing dyestuff.

Samples of the two film materials were treated for 8 minutes in a colour developer bath of the following composition:

|                                                 |    |
|-------------------------------------------------|----|
| 2 g. Calgon <sup>1</sup>                        | 25 |
| 2 g. sodium sulphite                            |    |
| 0.8 g. hydroxylamine sulphate                   |    |
| 75 g. potassium carbonate                       |    |
| 2 g. potassium bromide                          |    |
| 2.75 g. N,N-diethyl-p-phenylenediamine sulphate |    |
| 1 l. water                                      | 30 |

<sup>1</sup> A sodium hexametaphosphate-containing detergent as described, for example, on page 953 of the Merck Index, 7th Edition.

When the material had been bleached and fixed by the usual methods, no stain was detected in the two materials but the sharpness of the image in the material that contained the absorbing dyestuff according to the invention was much better.

#### Example 2

50 g. of 1,2-diaminonaphthalene-5,7-disulphonic acid was dissolved by heating in 350 ml. of water and 49 g. potassium acetate were added. 170 cc. of a 31% ferric chloride solution were stirred at 35° into this intensely coloured yellow solution. After stirring for one hour at room temperature, the precipitated dyestuff (B) was filtered off by suction, purified by digesting with 20% hydrochloric acid and dried at 70°. 27 g. of a dark green powder, soluble in water to give a brilliant blue-green solution were obtained.

A three layer positive colour film was built up as in Example 1, except that all the layers contained 0.6 g. of dyestuff (B) per kg. of emulsion, corresponding to about 120 mg. per m.<sup>2</sup> of film surface. A micro line screen was illuminated on to samples of this film and on to another film used for comparison which was made in the same way but without the addition of protective dyestuff (B). After developing the colour as in Example 1, the following fog densities were measured for the unilluminated areas:

|                                      | Blue-green | Magenta | Yellow |
|--------------------------------------|------------|---------|--------|
| Without absorbing dyestuff (B) ----- | 0.07       | 0.08    | 0.11   |
| With absorbing dyestuff (B) -----    | 0.07       | 0.09    | 0.10   |

On projecting the films and on microscopic interpretation of the screen images, the material without absorbing dyestuff gave a resolution of 140 lines/mm. whereas the material with absorbing dyestuff had a resolution of 165 lines/mm. and much better contrast.

#### Example 3

35.4 g. 1,2-diaminonaphthalene-3,6-disulphonic acid

and 29.4 g. potassium acetate were dissolved together in 200 ml. water. 32 g. of ferric chloride dissolved in 100 ml. water were added at 35° with stirring. The product was filtered after 15 minutes and the filtrate was treated with 1½ times its volume of alcohol and the precipitated dyestuff (C) was separated by suction filtration, washed with about 50 ml. of 96% alcohol and dried in a drying oven at 70°. 37 g. of a greenish black powder readily soluble in water to give a clear blue-green solution were obtained.

0.5 g. of this dyestuff was dissolved in 25 ml. water and added to 1 kg. of a gelatine-silver chloride emulsion which had been sensitised to red with dyestuff Rr 1953 and which contained 12 g. of the blue-green coupler 1-hydroxy-2-naphthoyl-4-sulpho-octadecylamide. This emulsion was cast as the uppermost layer over a layer consisting of a blue sensitive gelatine-silver bromide layer with yellow colour couplers on paper coated with barium sulphate and above it a green sensitive gelatine-silver chloride emulsion layer with magenta colour coupler. The same three layer element on a paper base but without the addition of absorbing dyestuff (C) was prepared for comparison. Samples of the two materials were treated for 5 minutes in the following dye developer baths:

|    |                                                              |
|----|--------------------------------------------------------------|
| 25 | 2 g. Calgon <sup>1</sup>                                     |
|    | 2 g. hydroxylamine sulphate                                  |
|    | 4 g. sodium sulphite                                         |
|    | 1 g. potassium bromide                                       |
|    | 100 g. potassium carbonate                                   |
| 30 | 5 g. N,N-dibutyl-p-phenylenediamine $\omega$ -sulphonic acid |
|    | 1 l. water                                                   |

<sup>1</sup> A sodium hexametaphosphate-containing detergent as described, for example, on page 953 of the Merck Index, 7th Edition.

After bleaching and fixing the samples in the usual way the following differences in fog density hardly perceptible with the naked eye were measured:

|                                      | Blue-green | Magenta | Yellow |
|--------------------------------------|------------|---------|--------|
| Without absorbing dyestuff (C) ----- | 0.15       | 0.13    | 0.18   |
| With absorbing dyestuff (C) -----    | 0.16       | 0.15    | 0.19   |

It will be clear to those skilled in the art that the praxis of our invention lends itself readily to a number of useful modifications in method, materials and so on. The photographic silver halide emulsions can be optically sensitised or unsensitised. The usual optical sensitising dyes for the red range of the visible spectrum can be used such as cyanines, merocyanines, complex (trinuclear) cyanines or merocyanines, styryls etc. In general the particular dyes according to the invention should have its maximum absorption in the same spectral region to which the sensitising dye sensitises the emulsion.

55 The dyestuffs can be used for silver chloride, bromide or iodide emulsions, or for emulsions containing mixtures of silver halides. Emulsions of silver chloride or silver chloro bromide are preferred. While our invention is particularly directed to the ordinary employed silver halide gelatine emulsions, binding agents other than gelatine, e.g., polyvinyl alcohol or cellulose materials, such as hydrolyzed cellulose acetate, carboxymethyl cellulose or the like which have no deleterious effect upon the light-sensitive materials, can be employed alone or in combination with gelatine.

The emulsions prepared in accordance with our invention can be coated in the usual manner upon any suitable support, e.g., cellulose acetate films, polycarbonate films, polystyrene films, polyester films etc.

We have found that the advantages of our invention are particularly outstanding when the support is paper or some other fibrous material which is more likely to adsorb stain than hydrophobic materials.

The silver halide emulsions according to the invention

can also contain such addenda as chemical sensitizers, e.g., sulfo sensitizers, various gold compounds, palladium compounds and the like; antifoggants, hardeners etc. The blue-green colour-coupler used in the emulsion according to the invention is not especially critical and is selected according to the requirements of the particular copying material in which the emulsion is to be used.

We claim:

1. A photographic silver halide gelatine emulsion optically sensitized to the red region of the spectrum containing from about 0.5 to 10 g. per mole of silver halide of a water soluble dye, said dye being a reaction product of ferric chloride with 1,2-diaminonaphthalene disulphonic acids, said reaction product having its maximum absorption in the red region of the spectrum.

2. A photographic silver halide gelatine emulsion according to claim 1, containing from about 0.5 to 10 g. per mole of silver halide, of the reaction product of ferric chloride with 1,2-diaminonaphthalene - 3,7-disulphonic acid.

3. A photographic silver halide gelatine emulsion according to claim 1, containing from about 0.5 to 10 g. per mole of silver halide, of the reaction product of ferric chloride with 1,2-diaminonaphthalene - 5,7-disulphonic acid.

4. A photographic silver halide gelatine emulsion according to claim 1, containing from about 0.5 to 10 g. per mole of silver halide, of the reaction product of ferric chloride with 1,2-diaminonaphthalene - 3,6-disulphonic acid.

5. A photographic element for subtractive colour photography comprising a support having coated thereon a plurality of silver halide emulsion layers, one of which is sensitive to the blue region of the spectrum and con-

tains a colour-forming compound capable of coupling with the oxidation products of a colour developer to produce a yellow image, one of which is sensitive to the green region of the spectrum and contains a colour-forming compound capable of coupling with the oxidation products of a colour developer to produce a magenta image and one of which is sensitive to the red region of the spectrum and contains (1) a colour-forming compound capable of coupling with the oxidation products of a colour developer to produce a cyan image and (2) from about 0.5 to 10 grams per mole of silver halide of a water soluble dye having its maximum absorption in the red-light region of the spectrum, said dye being a reaction product of ferric chloride with 1,2-diaminonaphthalene-disulphonic acid.

6. A photographic element according to claim 5, wherein in the support is paper and a silver halide emulsion layer closest to the support is a blue silver halide emulsion layer, the silver halide emulsion layer farthest from the paper support is a red sensitized silver halide emulsion layer and the green silver halide emulsion layer lies between the red sensitized silver halide emulsion layer and the blue sensitive silver halide emulsion layer.

25

#### References Cited by the Examiner

##### FOREIGN PATENTS

1,163,100 9/58 France.

##### OTHER REFERENCES

Sommer: *Chemicke Lisy*, vol. 52, pages 1485-1500 (1958).

NORMAN G. TORCHIN, Primary Examiner.